

# UNITED STATES PATENT OFFICE.

JOHN BARNES, OF BROOKLYN, NEW YORK, ASSIGNOR OF ONE-HALF TO PETER B. BIRD, OF NEW YORK, N. Y.

## BOILER COMPOUND.

1,181,562.

Specification of Letters Patent.

Patented May 2, 1916.

No Drawing. Application filed December 13, 1912, Serial No. 736,605. Renewed January 29, 1914. Serial No. 815,291.

*To all whom it may concern:*

Be it known that I, JOHN BARNES, a citizen of the United States, residing at Brooklyn, in the county of Kings and State of New York, have invented certain new and useful Improvements in Boiler Compounds, of which the following is a full, clear, and exact specification.

This invention relates to boiler compounds to prevent the formation of and to remove scale or incrustation formed by deposits of lime and magnesia salts, and to arrest and prevent objectionable corrosion, galvanic or electrolytic action.

Boiler compounds, as heretofore known, have been readily soluble powders, pastes or liquids, and considerable difficulty has been encountered in feeding them to boilers. Powders have had to be put into the boiler before steam was gotten up, or fed through a feed-cup. If put in before, it dissolved so quickly as to cause foaming, and if attempted to be fed through a feed-cup, it was found that the dry powder would attack the metal, and cause the cocks to stick, with liability of breakage, and danger of scalding the attendants. In powders containing mercury, especial difficulty is encountered, because the mercury would sink to the bottom, and not be circulated with the other ingredients throughout the surface of the boiler, on account of its specific gravity. Liquids or pastes containing mercury are subject to the same difficulties.

It is the object of this invention to provide a boiler compound containing mercury, which can be made up in hard form, and, when put into the boiler, will dissolve slowly and hold the mercury in such state of fine sub-division, that it can be carried by the circulation to all parts of the boiler, without settling. To this end, I form my compound as a hard, agglomerated cake which the water under heat and pressure gradually dissolves, thereby neutralizing acids or oils in the water, and at the same time setting freely molecularly fine quantities of metallic mercury, which spreads in thin film over the surface of the tubes and sheets. The heat and pressure cause the mercury to form a glazed metallic surface in contact with the iron, and permits efficient transmission of heat to the water. The use of mercury has heretofore been proposed

to prevent incrustation, but it has always been introduced in such form that it tended to collect in a pool at the bottom of the boiler, thereby becoming useless. By amalgamating mercury with an alkali metal, such for example as sodium, the tendency of the mercury to form a galvanic couple with the iron in acid waters, is neutralized, as the amalgam is electro positive to iron or steel under heat and pressure, thereby preventing electrolytic action on the iron. The mercury is thus polarized, relatively to iron or steel, and protects the iron from attack by electrolysis or galvanic action, as well as, in connection with the other ingredients, forming a protective, heat conducting coating.

In carrying out my invention, I form an amalgam of mercury and an alkali metal, such for example as sodium. I preferably select proportions such that the amalgam will have to be pulverized into impalpable powder before being mixed with the other ingredients. As an example of an efficient compound I may employ fifteen parts of amalgam, ten parts of kerosene emulsified with oil containing as low content of free fatty acid as possible, such as whale or seal oil, fifteen parts of sodium hydrate, twenty-five parts of dextrin or other suitable carbohydrate, ten parts of tannin, kutch, or other tannin containing material, and fifteen parts of tri-sodium phosphate, and water to mix, ten parts. The ingredients are thoroughly mixed, and then agglomerated under pressure into a hard cake. These proportions may be varied within wide limits according to the character of the water used in the boiler; other alkaline salts may in some cases be preferred or may be added to the sodium phosphate, such as soda ash or the alkaline chromates. The hard cakes of my compound may be introduced into the boiler in containers, and will dissolve gradually without causing the mercury to settle. The several ingredients are therefore slowly set free and enter into circulation with the feed water, exerting a beneficial action on the prevention and removal of the calcareous scale. The amalgam as slowly freed is broken up by the affinity of water for sodium which goes into solution leaving the mercury with the emulsified kerosene to be distributed in the boilers in a molecularly

fine form. Kerosene is very useful for its effect on sulfate of lime and magnesia which tend to form scale, as well as neutralizing or dissolving any grease that may be in the boiler, so that a clean metal surface may be exposed for holding the mercury. As well known, kerosene alone would have so low a boiling point that it would volatilize under the heat in boilers and would rise into the steam drum and escape, but by being emulsified with an oil of high boiling point it intimately mixes with the water and is much slower to volatilize; its emulsification also facilitates the compounding into the cake form. The sodium hydrate or caustic soda neutralizes any acidity of the feed water and combines with oil or grease in the boiler or feed water to form a soluble soap and to cut the scale and cleanse the underlying metal. The dextrin has a beneficial action on the sulfates and acts as a binder in forming and maintaining the compound in a solid state. The tri-sodium phosphate neutralizes the corrosive action produced by many feed waters. The tannin or kutch arrests foaming common in boilers when alkaline waters have to be used, and also has a beneficial effect on carbonates of lime or magnesia. In addition to the dextrin or in substitution therefor I sometimes use other gums or sugars as a soluble binder. The mercury forms an acid proof, heat conducting coating. The polarized mercury amalgam has no effect upon brass or copper under water. The emulsified kerosene may be formed, according to one preferred method, by saponifying whale or seal oil, or green soap made therefrom, preferably mixed with gelatin or similar substance, then adding the kerosene oil to the same, and then working the whole with the remaining ingredients to form the slowly soluble boiler compound of the invention. The green soap should preferably be free from free fatty acid, glycerin, stearin, or like substance. Usually, the kerosene is added by small quantities at a time

to the mass containing green soap, water and gelatin, the kerosene being thoroughly mixed by active stirring.

My invention has proven to be especially well adapted to locomotive boilers which on account of their small steam space and high working pressure foam or prime very quickly and owing to the use of copper expansion rings are more liable to galvanic action causing pitting and grooving on both plates and tubes. By reason of the hard, slowly soluble characteristics of my improved boiler compound, it is possible to place in a boiler at one time, a sufficient quantity to last two or three months without attention, or without causing foaming, thereby obviating the expense and trouble of daily feeding of boiler compound, and also avoiding the necessity of frequent washing out and opening the boiler.

Having thus described my invention, I declare that what I claim as new and desire to secure by Letters Patent, is:—

1. A hard, slowly soluble boiler compound containing amalgam, and emulsified kerosene.

2. A hard, slowly soluble boiler compound containing amalgam and emulsified kerosene distributed in a soluble binder.

3. A hard, slowly soluble boiler compound containing a mixture of sodium amalgam, tannin and emulsified kerosene, distributed in a soluble binder.

4. A boiler compound slowly soluble in water having the physical characteristics of a hard cake, comprising a soluble binder containing alkali together with finely subdivided amalgam rendered electro-positive to iron and steel and distributed throughout said hard slowly soluble cake.

In testimony whereof I affix my signature in presence of two witnesses.

JOHN BARNES.

Witnesses:

PETER A. ROE,  
HELEN C. EGAN.